

## UNITED STATES PATENT OFFICE.

ROBERT F. RAYNOR, OF ST. PAUL, MINNESOTA.

## POLISHING COMPOSITION.

No Drawing.

Application filed February 10, 1928. Serial No. 253,527.

The present invention relates to a new and improved polish for furniture and vehicles such as automobiles, to a dressing for leather, and a cleansing and polishing agent for glass, 5 brass, nickel and enamel.

The polish made in accordance with the present invention is very easily applied to the article to be treated by simply applying the liquid to the article and rubbing with a soft 10 cloth, it being an important feature of the composition of the present invention that very little labor is required to produce a polished surface which does not produce finger marks upon the touch of the fingers with the 15 polished surface, or other marks upon contact of other bodies with the polished surface. So far as a polished surface is concerned, a substantially fixed gloss is obtained, which dulls very slowly and is not impaired by contact of various bodies therewith. The known 20 polishes with a wax base usually leave a velvet or filmy coating on the finish that shows up finger print marks and the marks of everything that comes in contact with the surface polished with them. This detrimental effect is eliminated by the polish of the present invention. Polishes with a wax base usually require a great expenditure of labor in bringing 25 about the proper finish and this fact alone is a deterrent to their use. In contradistinction to this latter disadvantage, the polish of the present invention produces a highly lustrous and permanent finish with very little or no rubbing after it has been uniformly applied to the surface to be polished or treated.

In the above indicated respects, the composition of the present invention is also a material improvement over the oily polishes which also require much labor to rub the 40 surface dry to which they are applied, if in fact they can be rubbed dry.

These wax and oily polishes of the prior art have the further disadvantage that their finished surfaces is filmy or sticky, which condition induces the collection of dust and lint. The objectionable properties are entirely absent when the composition of the present 45 invention is used.

There are also other polishes of the prior 50 art which are nothing more than cheap varnishes which are designed to dry quickly and therefore require very little rubbing with a cloth. However this type of compositions cover up the grain of the wood and usually 55 leave a sticky foundation for dust, since the

drying is not complete. Furthermore cracking of such an added layer usually occurs and impairs the article to which the composition is applied. The composition of the present invention does away completely with the defects of the varnish type of polish. 60

From the foregoing it will appear that the composition of the present invention presents new and improved properties which enable the defects in known compositions of a similar 65 nature to be overcome.

The composition of the present invention cleans as it does its work, does not crack the finish, leaving dull finish in its original state and giving a high polish and beautiful lustre 70 to highly polished surfaces.

In compounding the composition of the present invention the following procedure may be adopted: Dissolve 15 grains of pulverized gum sandarac in 4 $\frac{3}{4}$  ounces ethyl 75 alcohol or denatured alcohol. The gum sandarac is preferably pulverized to aid in the preparation of the invention as it dissolves more quickly in the pulverized state than in the state of lumps or tears. To this 80 solution 4 $\frac{3}{4}$  ounces of cider vinegar or a corresponding amount of acetic acid is added. This causes a precipitation of a white chalky mass representing certain components of the gum sandarac which do not remain in solution and which it is desired to separate. 2 $\frac{1}{4}$  85 ounces of paraffin oil are then added and then 4 $\frac{3}{4}$  ounces of benzine or benzene.  $\frac{1}{2}$  ounce of citronella may be added to perfume the product if desired. The mixture is well 90 stirred or shaken and allowed to stand about 24 hours or more, and then strained through two or three thicknesses of cheese cloth for taking out the white chalky sediment, retaining the desired component of the gum 95 sandarac. If desired the chalky precipitate may be removed from the mixture at the time of its formation and before adding the other ingredients of the composition. By permitting the composition to stand for 24 hours 100 or more the composition becomes clean and clear and more suitable for commercial use and sale.

In the use of acetic acid instead of vinegar care must be exercised not to use too much 105 as it is so much stronger than vinegar. If too much acetic acid is employed the tendency is to leave a filmy smoky effect, which is generally avoided by using the quantity of cider vinegar indicated. 110

In the accompanying claims the term benzine is used in the sense of including benzine and benzene.

Having described my invention what I claim is:

1. A composition comprising benzine, paraffin oil, and the composition obtained by precipitating a solution of gum sandarac in alcohol by means of acetic acid and separating 10 of the white chalky precipitate therefrom.
2. A composition of matter comprising

the following ingredients in substantially the proportions given:  $4\frac{3}{4}$  ounces benzine,  $2\frac{1}{4}$  ounces paraffin oil, and the product obtained by precipitating a solution of 15 grains of gum sandarac in  $4\frac{3}{4}$  parts of alcohol by means of  $4\frac{3}{4}$  ounces of vinegar and separating 15 of the white chalky precipitate therefrom.

In testimony whereof I affix my signature.

ROBERT F. RAYNOR.